

Oct. 14, 1958

O. L. RIGGS, JR.

2,856,358

METHOD OF INHIBITING CORROSION

Filed May 2, 1955

2 Sheets-Sheet 1



FIG. 1

INVENTOR.  
OLEN L. RIGGS, JR.

BY

*Floyd Trimble*

ATTORNEY

Oct. 14, 1958

O. L. RIGGS, JR

**2,856,358**

## METHOD OF INHIBITING CORROSION

Filed May 2, 1955

2 Sheets-Sheet 2



FIG. 2

INVENTOR.  
OLEN L. RIGGS, JR.

BY

Floyd Trimble

ATTORNEY

1

2,856,358

## METHOD OF INHIBITING CORROSION

Olen L. Riggs, Jr., Ponca City, Okla., assignor to Continental Oil Company, Ponca City, Okla., a corporation of Delaware

Application May 2, 1955, Serial No. 505,469

9 Claims. (Cl. 252—8.55)

This invention relates to retarding or the prevention of corrosion in oil wells and connecting pipe lines in intermediate storage to the refinery for crude oil. More particularly, I have found that an oil-soluble substituted glyoxalidine, also known as imidazoline salt of an alkaryl sulfonic acid, when added to well fluids in minor proportions acts to inhibit the rusting or corrosion of the metallic equipment used in the well due to hydrogen sulfide and carbon dioxide environments.

Considerable corrosion takes place in the metallic equipment of practically all oil wells and in certain environments, corrosion may reach costly proportions. For example, casing, tubing, sucker rods, and lead lines are particularly subject to corrosion. The sucker rods and sucker rod boxes which operate under heavy cyclic load conditions are especially susceptible to failure through corrosion fatigue. As a result of corrosion, costs of operations are greatly increased because of the necessity of pulling tubing and sucker rods for repair or replacement. In addition, indirect costs in terms of production losses while shut down for repair or replacement are high.

It is, therefore, a principal object of this invention to provide a method of preventing corrosion in oil wells which is effective and economical. Another object of my invention is to provide a substance which can be added to the oil well which will control corrosion and particularly will reduce pitting without any adverse effects on the crude oil. Other objects and advantages will be apparent from the following description.

In brief, I have discovered that the addition of a minute quantity of a substituted glyoxalidine salt of an alkaryl sulfonic acid to an oil well containing fluids which cause corrosion is effective in inhibiting or preventing corrosion of the metal exposed to such fluids.

I have found that the corrosive effects of the fluids on metallic surfaces can be substantially reduced and in many cases practically eliminated by the introduction of an exceedingly small quantity of an oil-soluble substituted glyoxalidine salt of an alkaryl sulfonic acid into the well. The particular substituted glyoxalidines or imidazolines useful in my invention are hydroxy compounds. The inhibitor may be added to the well fluids by any conventional method; usually, by merely injecting the desired amount of the inhibitor into the well. As another method of introducing the inhibitor into the well, a tubing of relatively small diameter may be run down the center of the production tube of the well to approximately the bottom end thereof and a solution of the inhibitor may be pumped through the small diameter tubing so as to enter the well stream near the bottom of the well tube. The rising turbulent flow will then carry the injected inhibitor up through the tube. Obviously the corrosion inhibitor may be added or introduced into the well by other means or methods depending in part on whether the wells are operated through the casing or through tubing disposed in such casings. Also, it is clear that the inhibitors may be introduced into the top of the well and allowed to

2

flow down or may be forced through any given point or points in the well at which the inhibitor then can come in contact with the turbulent up-going fluid mixture which, as stated, would cause metal corrosion but for the presence of the corrosion inhibitors of this invention.

5 The effective and preferred proportions of my inhibitor are in the range approximately 2 to 500 and 25 to 100 parts per million of well fluid respectively; namely, crude oil in brine. After separating the brine from the crude oil, the resulting crude oil exhibits favorable corrosion inhibiting properties when transported through connecting pipe lines to the refinery.

10 The corrosion inhibitors of this invention may be introduced into the system as such or they may be dissolved in a suitable solvent such as mineral oil, crude oil, kerosene, gasoline, organic esters, alcohols, ketones, or even water. Although any solvent which is non-reactive with the corrosion inhibitor may be employed, kerosene or a light hydrocarbon fraction is preferred as the particular solvent. When a solvent is used, it is preferred to use a concentration of corrosion inhibitor varying from about 25 to 40 percent.

15 The substituted imidazolines useful in my invention are 1-hydroxy-alkyl-2-long chain alkyl imidazolines having the general formula:



25 where R is an alkyl radical containing from 11 to 17 carbon atoms, and R' and R'' are either the same or different and are selected from the group consisting of hydrogen and an alkyl group having from about 6 to 30 carbon atoms and x is an integer varying from 1 to 3. If both R' and R'' are alkyl groups, the total number of carbon atoms in those groups would vary from 12 to 18. 1-hydroxy-alkyl-2-long chain alkyl imidazolines are prepared by reacting a monocarboxylic acid or ester with a diamine containing a hydroxy group at an elevated temperature, generally in the range of about 230° C. or higher at which temperature water is evolved and ring closure effected. Specific instructions for preparing these compounds are given in U. S. Patent 2,267,965 issued December 30, 1941, to Alexander L. Wilson, and by Hofmann, Journal of Organic Chemistry 12, 577 (1947).

30 Suitable 1-hydroxyalkyl-2-long chain alkyl imidazolines for use in the improved corrosion inhibitors of this invention may be prepared by the reaction of a long chain fatty acid or ester and a hydroxylalkyl ethylene diamine. 35 Long chain fatty acids such as lauric acid, tridecanoic acid, myristic acid, oleic acid, stearic acid, palmitic acid, linoleic acid, linolenic acid, erucic acid, tall oil fatty acid, oxidized petroleum wax fractions, acid from oxidized "oxo" reaction products, etc.

40 Hydroxylalkyl ethylene diamines with which the long chain fatty acid may be reacted to yield substituted imidazolines suitable for this invention include: hydroxymethyl ethylene diamine, hydroxyethyl ethylene diamine, and the various hydroxy propyl ethylene diamines such as 1(3-hydroxypropyl) ethylene diamine, 1(2-hydroxypropyl) ethylene diamine, and (2-hydroxypropyl) ethylene diamine.

45 The preparation of 1-hydroxyalkyl-2-long chain alkyl imidazolines is exemplified by the reaction between stearic acid and hydroxyethyl ethylene diamine. By heating at 250° C., one mole of stearic acid with one mole of

hydroxyethyl ethylene diamine, two moles of water are liberated and 1-hydroxyethyl-2-heptadecyl imidazoline is formed in accordance with the equation:



Examples of other 1-hydroxyalkyl-2-long chain alkyl imidazolines include:

1-hydroxymethyl-2-undecyl imidazoline  
1-hydroxyethyl-2-undecyl imidazoline  
1-hydroxypropyl-2-undecyl imidazoline  
1-hydroxyethyl-2-dodecyl imidazoline  
1-hydroxymethyl-2-tridecyl imidazoline  
1-hydroxymethyl-2-heptadecenyl imidazoline  
1-hydroxyethyl-2-heptadecenyl imidazoline  
1-hydroxypropyl-2-heptadecenyl imidazoline  
1-hydroxymethyl-2-heptadecyl imidazoline  
1-hydroxyethyl-2-heptadecyl imidazoline  
1-hydroxyethyl-2-pentadecyl imidazoline  
1-hydroxypropyl-2-pentadecyl imidazoline  
1-hydroxyethyl-2-heptadecadienyl imidazoline

Suitable alkaryl sulfonic acids are those obtained by the sulfonation of alkaryl hydrocarbons, which in turn are produced by the alkylation of an aromatic hydrocarbon such as benzene, toluene, xylene, cumene, and similar aromatic hydrocarbons. Straight or branched chain olefins, alcohols, or halides having from about 6 to about 30 carbon atoms and preferably from about 12 to about 18 carbon atoms are used as the alkylating agents. As to the olefins, those may be obtained by the polymerization of low molecular weight olefins such as ethylene, propylene, and mixtures thereof or may be obtained by the cracking or hydroforming of hydrocarbons such as wax, kerosene, or other petroleum fractions. Suitable alkaryl sulfonic acids for use in my invention are those having molecular weights within the range of about 400-550. These acids are obtained by sulfonating alkaryl hydrocarbons of the proper molecular weight. A particular useful sulfonic acid is postdodecylbenzene sulfonic acid which is obtained by sulfonating the detergent alkylate known as postdodecylbenzene. Postdodecylbenzene consists of monoalkylbenzenes and dialkylbenzenes in the approximate ratio of 2:3. Its typical physical properties are as follows:

|                            |             |        |
|----------------------------|-------------|--------|
| Specific gravity at 38° C  |             | 0.8659 |
| Average molecular weight   |             | 365    |
| Percent sulfonatable       |             | 88     |
| A. S. T. M., D-158 Engler: |             |        |
| I. B. P                    | ° F         | 647    |
| 5                          | ° F         | 682    |
| 50                         | ° F         | 715    |
| 90                         | ° F         | 760    |
| 95                         | ° F         | 775    |
| F. B. P                    | ° F         | 779    |
| Refractive index at 23° C  |             | 1.4900 |
| Viscosity at:              |             |        |
| —10° C                     | centipoises | 2800   |
| 20° C                      | do          | 280    |
| 40° C                      | do          | 78     |
| 80° C                      | do          | 18     |
| Aniline point              | ° C         | 69     |
| Pour point                 | ° F         | —25    |

In addition to the sulfonic acid obtained by sulfonating postdodecylbenzene, other alkaryl sulfonic acids have been used wherein the molecular weight of the acid has varied from about 320 to over 600. Dodecylbenzene sulfonic acid and diwaxbenzene sulfonic acid are examples of acids having molecular weight of 320 and over.

600 respectively. The molecular weight of diwaxbenzene sulfonic acid is approximately 630 and is obtained by alkylating benzene with chlorowax.

The alkaryl hydrocarbons so obtained may be sulfonated by any conventional sulfonating method which procedures are well known to those skilled in the art; however, I prefer the method disclosed in the co-pending application entitled "Method of Sulfonating Alkyl Aromatic Hydrocarbons," by Luntz and Popovac, filed December 8, 1953, Serial No. 396,822, now U. S. Patent 2,768,199, which disclosure is made a part of this application.

Following the production of the sulfonic acid as described above, the salt may be formed by mixing equal molecular proportions of the imidazoline with the alkaryl sulfonic acid. The imidazoline may be added to the sulfonic acid or conversely the sulfonic acid may be added to imidazoline. The reaction is generally very rapid and as a consequence the reaction is 100 percent complete by the time the components are mixed, however, if necessary external heating or cooling may be employed for an additional time to complete the reaction.

In addition to the uses enumerated above, my inhibitors  
25 may be used effectively to inhibit corrosion in tankers  
carrying crude oil or refined petroleum products. They  
are also valuable in preventing corrosion of pipe line  
carrying either crude oil or petroleum refined products.

In order to disclose the nature of the present invention still more clearly the following illustrative examples will be given. It is to be understood, however, that the invention is not to be limited to the specific conditions or details set forth in these examples except in so far as such limitations are specified in the appended claims.

The efficiencies of the various inhibitors were determined both in hydrogen sulfide and carbon dioxide environments. The methods used are as described under Procedures A and B below.

## PROCEDURE A

Efficiencies of corrosion inhibitors in a hydrogen sulfide environment were compared by determining the percent protection given a mild carbon steel test coupon subjected to corrosive conditions in the presence of the corrosion inhibitor in the equipment illustrated in Fig. 1. A large-mouth bottle of about 250 ml. capacity was charged with 150 ml. of Arbuckle brine and 50 ml. of kerosene containing the corrosion inhibitor being tested. The bottle was agitated to distribute the corrosion inhibitor between the two phases, a weighed 1-inch by 3-inch 10-20 mild carbon steel coupon inserted, and bottle stopper fitted on. Hydrogen sulfide was bubbled through the solution at a rate of about 12 ml. per second. After about 18 hours, the coupon was removed from the bottle, descaled by scrubbing with a nylon bristle brush and a cleaning powder, weighed and its loss in weight determined. The same technique was followed to obtain a blank in the absence of corrosion inhibitor. The percent protection was calculated as follows:

$$P.C.P. = \frac{(Wb_i - Wb_f) - (Wc_i - Wc_f)}{(Wb_i - Wb_f)} \times 100$$

### whereas

P. C. P.=percent protection afforded by inhibitor.  
 $Wb_i$ =initial weight of coupon subjected to test in the  
absence of inhibitor.

$W_{b_f}$  = final weight of coupon subjected to test in the absence of inhibitor.

$W_{C_i}$ —initial weight of coupon subjected to test in presence of inhibitor.

$W_{C_f}$ =final weight of coupon subjected to test in the presence of inhibitor.

## PROCEDURE B

Equipment suitable for determination of corrosion in an atmosphere of carbon dioxide is shown in Fig. 2. Vessel A is equipped with a motor D for rotating a coupon holder C holding coupon P. Provisions B and E provide for introducing and exhausting carbon dioxide that has been metered in flow meter F and saturated with water vapor in wetting vessel G. H is a thermometer for indicating the temperature of the fluids undergoing test and J is a means for withdrawing samples of fluid undergoing test. Q is a vessel attached to the glass jar A and is provided with a screw cap R. Vessel Q fits over trap door S. The purpose of this vessel is for inserting the coupon P into the glass jar A. T indicates a bearing through which the shaft of motor D passes. Pump supplies means for maintaining immiscible fluids in dispersed state. Corrosion rate in units of mil penetration per year is calculated as follows:

$$M. P. Y. = \frac{1000(W_i - W_f)}{g^A t}$$

where:

M. P. Y.=mils penetration per year.

$W_i$ =initial weight of coupon in grams.

$W_f$ =final weight of coupon in grams.

$g$ =specific weight of coupon in grams per cubic inch.

$A$ =area of coupon in square inches.

$t$ =duration of corrosion test in years.

The present invention may be clearly understood from the following examples which are given by way of illustration only and are not intended to be considered as a limitation of the invention.

## Example 1

One molecular weight of imidazolines sold by the Alrose Chemical Company of Providence, Rhode Island, as Amine C, Amine O, and Amine S and having the structure,



in which R is undecyl, heptadecenyl, and heptadecyl and molecular weights are 276, 355, and 360, respectively, was added to one molecular weight of postdodecylbenzene sulfonic acid having a molecular weight of 440 and obtained by the sulfonation of the still bottoms remaining after distilling the alkylation product of benzene with tetrapropylene up to 205° C. at 20 mm. pressure. The 1-hydroxyethyl-2-long chain alkyl imidazoline polydodecylbenzene sulfonate obtained was tested as a corrosion inhibitor in accordance with Procedure A. The results are given in the following Table 1.

TABLE 1.—PERCENT PROTECTION OFFERED BY VARIOUS CONCENTRATIONS OF IMIDAZOLINE SULFONATES

| Imidazoline Sulfonate Salt |                                   | Concentration—p. p. m. |    |    |    |     |
|----------------------------|-----------------------------------|------------------------|----|----|----|-----|
| Imidazoline                | Sulfonic Acid                     | 5                      | 10 | 25 | 50 | 100 |
| Amine C                    | PDBSO <sub>3</sub> H <sup>1</sup> | 76                     | 84 | 91 | 91 | 91  |
| Amine O                    | PDBSO <sub>3</sub> H <sup>1</sup> | 70                     | 71 | 88 | 90 | 96  |
| Amine S                    | PDBSO <sub>3</sub> H <sup>1</sup> | 86                     | 92 | 94 | 95 | 97  |

<sup>1</sup> Postdodecylbenzene sulfonic acid having molecular weight of 440.

## Example 2

The substitution of other alkyl aromatic sulfonic acids having a molecular weight of about 400 to about 550 for the postdodecylbenzene sulfonic acid of molecular weight 440 used in Example 1 gives salts offering corrosion inhibition of the same order as the salts listed in Table 1.

## Example 3

On substitution of dodecylbenzene sulfonic acid having a molecular weight of 320 and obtained by sulfonating the alkylation product of benzene with tetropropylene for postdodecylbenzene in Example 1, a salt was obtained with Amine S which gave about 70 percent protection at 100 p. p. m. concentration.

## Example 4

On substitution of diwaxbenzene sulfonic acid of molecular weight 630 and obtained by alkylating benzene with chlorowax for postdodecylbenzene in Example 1, a salt was obtained with Amine S which gave about 50 percent protection at 100 p. p. m. concentration.

## Example 5

One molecular weight of Amine 230, a product of Carbide and Carbon Chemical Company and being 1-aminoethyl-2-heptadecyl imidazoline was added to molecular weight of postdodecylbenzene sulfonic acid and dodecylbenzene sulfonic acid. The salts obtained were tested as a corrosion inhibitor in accordance with Procedure A. The results are given in Table 2.

TABLE 2.—PERCENT PROTECTION OFFERED BY VARIOUS CONCENTRATIONS OF 1-AMINOETHYL IMIDAZOLINE SULFONATES

| Imidazoline Sulfonate Salt |                                   | Concentration—p. p. m. |    |    |    |     |
|----------------------------|-----------------------------------|------------------------|----|----|----|-----|
| Imidazoline                | Sulfonic Acid                     | 5                      | 10 | 25 | 50 | 100 |
| Amine 230                  | PDBSO <sub>3</sub> H <sup>1</sup> | 36                     | 63 | 76 | 78 | 83  |
| Amine 230                  | DBSO <sub>3</sub> H <sup>2</sup>  | 4                      | 48 | 59 | 59 | 70  |

<sup>1</sup> Postdodecylbenzene sulfonic acid.

<sup>2</sup> Dodecylbenzene sulfonic acid.

Examples 1 to 5 were repeated except that the corrosion tests were conducted in a carbon dioxide environment in accordance with Procedure B rather than in a hydrogen sulfide environment. The results obtained as to the amount of protection afforded by the imidazoline derivatives in the carbon dioxide environment were similar to that afforded in the hydrogen sulfide environment. Examples 1 and 2 were repeated with the exception that 45 the corrosion tests were conducted in an environment comprising both carbon dioxide and hydrogen sulfide. The protection afforded by the imidazoline derivatives in the presence of the two gases was excellent.

A comparison of the data of Tables 1 and 2 show that 50 of the substituted imidazoline salts those prepared from the 1-hydroxy-alkyl-2-long chain alkyl imidazolines are more effective as inhibitors than those prepared from the 1-amino-alkyl-2-long chain alkyl imidazolines. Examples 1, 2, 3, and 4, show that the salts formed from 55 alkaryl sulfonic acids having a molecular weight within the range of 400-550 are more effective as inhibitors than those prepared from alkaryl sulfonic acids having molecular weights outside that range.

What is considered new and inventive in the present invention is defined in the hereunto appended claims, it being of course understood that equivalents known to those skilled in the art are to be construed as within the scope and purview of the claims.

I claim:

1. The method of inhibiting corrosion of ferrous metals in contact with corrosive fluids which comprises the addition to said corrosive fluids of an amount within the range of 2 to 500 parts per million of the corrosive fluids contacted an oil-soluble salt, said salt being the reaction product of 1-hydroxy-alkyl-2-long chain alkyl imidazoline and an alkaryl sulfonic acid wherein the alkaryl sulfonic acid has a molecular weight within the range of about 400 to 550.

2. The method of inhibiting corrosion of ferrous metals in contact with corrosive fluids which comprises

the addition to said corrosive fluids of an amount within the range of 25 to 100 parts per million of the corrosive fluids contacted an oil-soluble salt, said salt being the reaction product of 1-hydroxy-alkyl-2-long chain alkyl imidazoline and an alkaryl sulfonic acid wherein the alkaryl sulfonic acid has a molecular weight within the range of about 400 to 550.

3. The method of claim 1 wherein the corrosive fluids contain carbon dioxide.

4. The method of claim 1 wherein the corrosive fluids contain hydrogen sulfide.

5. The method of inhibiting corrosion of ferrous metals in contact with corrosive fluids which comprises the addition to said corrosive fluids of an amount within the range of 2 to 500 parts per million of the corrosive fluids contacted an oil-soluble salt, said salt being the reaction product of 1-hydroxyethyl-2-undecyl imidazoline and an alkaryl sulfonic acid wherein the alkaryl sulfonic acid has a molecular weight within the range of about 400 to 550.

6. The method of inhibiting corrosion of ferrous metals in contact with corrosive fluids which comprises the addition to said corrosive fluids of an amount within the range of 2 to 500 parts per million of the corrosive fluids contacted an oil-soluble salt, said salt being the reaction product of 1-hydroxyethyl-2-heptadecyl imidazoline and an alkaryl sulfonic acid wherein the alkaryl sulfonic acid has a molecular weight within the range of about 400 to 550.

7. The method of inhibiting corrosion of ferrous metals in contact with corrosive fluids which comprises

the addition to said corrosive fluids of an amount within the range of 2 to 500 parts per million of the corrosive fluids contacted an oil-soluble salt, said salt being the reaction product of 1-hydroxyethyl-2-heptadecyl imidazoline and an alkaryl sulfonic acid wherein the alkaryl sulfonic acid has a molecular weight within the range of about 400 to 550.

8. The method of claim 1 wherein the alkaryl sulfonic acid is postdodecylbenzene sulfonic acid.

9. The method of inhibiting corrosion of ferrous metals in contact with corrosive fluids containing carbon dioxide and hydrogen sulfide which comprises the addition to said corrosive fluids of an amount within the range of 2 to 500 parts per million of the corrosive fluids contacted an oil-soluble salt, said salt being the reaction product of 1-hydroxy-alkyl-2-long chain alkyl imidazoline and an alkaryl sulfonic acid wherein the alkaryl sulfonic acid has a molecular weight within the range of about 400 to 550.

20

#### References Cited in the file of this patent

#### UNITED STATES PATENTS

|    |           |                      |               |
|----|-----------|----------------------|---------------|
| 25 | 2,466,517 | Blair et al. _____   | Apr. 5, 1949  |
|    | 2,468,163 | Blair et al. _____   | Apr. 26, 1949 |
|    | 2,493,483 | Francis et al. _____ | Jan. 3, 1950  |
|    | 2,583,399 | Wachter et al. _____ | Jan. 22, 1952 |
| 30 | 2,671,757 | Wisherd _____        | Mar. 9, 1954  |
|    | 2,785,127 | Shock et al. _____   | Mar. 12, 1957 |